

## UNITED STATES PATENT OFFICE.

JOSEPH R. COOLIDGE, 3D, OF BROOKLINE, MASSACHUSETTS, ASSIGNOR TO MONTAN, INC., OF BOSTON, MASSACHUSETTS, A CORPORATION OF MASSACHUSETTS.

## IMPREGNATED WOOD AND PROCESS OF TREATING WOOD.

No Drawing.

Application filed February 2, 1925. Serial No. 6,463.

*To all whom it may concern:*

Be it known that I, JOSEPH R. COOLIDGE, 3d, a citizen of the United States, residing at Brookline, in the county of Norfolk and State of Massachusetts, have invented certain new and useful Improvements in Impregnated Woods and Processes of Treating Woods, of which the following is a specification.

10 This invention relates to the treatment of wood with materials designed to improve its characteristics. It is the general object of the invention to increase the durability of wood, to eliminate certain of its objectionable properties, and to impart to it qualities which will increase its usefulness.

While wood has always been used very extensively in a great many industries, it possesses, nevertheless, certain objectionable characteristics such, for example, as its susceptibility to decay and its tendency to shrink and swell with changing moisture conditions. While these characteristics are well known and widely recognized, and wood is very generally used notwithstanding them, still they do limit seriously the extent to which wood can be used for some purposes, particularly since the price of desirable woods has become so high. This is well illustrated in the use of wooden poles by the telegraph, telephone, and electric light companies to support the wires which transmit electrical energy. Usually the more resistant woods, such as cedar and chestnut, are used for this purpose, but such poles only last on an average from eight to twelve years. The less resistant woods have an even shorter life. When these woods were very abundant the short life of such poles was not a particularly serious factor, but today the chestnut growth suitable for poles has almost entirely disappeared from the United States and cedar poles are now being shipped from the Pacific Coast States to supply the eastern market. Twenty years ago chestnut poles of a standard size could be purchased freely in the eastern States for about five dollars per pole. Today such poles are very scarce and a western cedar pole of the same dimensions commands a price of approximately twenty-five dollars in the eastern market. Furthermore, the labor expense involved in re-setting a pole has increased tremendously. Conse-

quently, the short life of wooden poles is a very important factor to the electric light, 55 telegraph and telephone companies.

The readiness with which wood absorbs water and gives it up, with the consequent swelling and shrinking of the wood, is also an objectionable characteristic of this material. This is true, for example, in using wood in the making of patterns for castings, in lasts for the manufacture of shoes and other footwear, and in furniture where the shrinking and swelling of the wood causes 60 the furniture to crack and opens the joints. It is further objectionable in flooring, in wooden boats where the shrinking and swelling must be taken care of by calking, and in many other uses. 70

It has been proposed heretofore to overcome certain of these objections, particularly that of decay, by saturating the wood with toxic preservatives. The most satisfactory preservative for wood so far discovered is 75 creosote, and while this is widely used on railroad ties, piles and the like, it exudes freely from the wood at atmospheric temperatures and therefore renders the wood totally unfit for other uses where it must be handled or where it comes in contact with the person or clothing of individuals. Much of the creosote also is lost after a relatively few years when the creosoted timber is exposed to the weather. That is, the creosote 80 exudes from the cells of the wood in warm weather, particularly under the action of the sun, and the creosote so exposed on the surface of the wood is washed away by rains and its effectiveness is lost. 85

It has also been proposed to impregnate wood with other materials which are known to be water-resistant, such for example, as the asphalts, resins and gums, but none of these materials becomes sufficiently fluid at 90 the temperatures to which wood can be subjected without injuring its fibre to permit them to be introduced into the tracheids of the wood. While they might be so introduced by solution in solvents, this procedure 100 involves additional practical difficulties and increases the expense of the treatment to such a degree that it is not feasible for most purposes.

The present invention deals especially 105 with the problem of preserving wood against

decay and making it substantially impervious to moisture.

To accomplish this object requires the impregnation of the wood with a material having the following characteristics:

First: It must be waterproof. The fibre of the wood itself is not waterproof, but, on the contrary, has a marked affinity for water. Consequently, in order to render the wood waterproof the fibre of the wood must be protected by a waterproof material.

Second: It must be hard and devoid of any tackiness or greasiness at the maximum temperature to which the wood naturally will be subjected while in use. Wood exposed to the sun on summer days may attain a temperature of 130° F. or 140° F. Consequently, the impregnating material must be able to withstand this temperature without becoming sticky or greasy.

Third: The material must become so fluid at 250° F. or lower, that it can be introduced into the tracheids of the wood so that a thorough impregnation of the wood can be effected. The temperature limit of 250° F. is fixed by the fact that if wood is exposed to a substantially higher temperature for any great length of time its structure is weakened. The impregnation process, therefore, should be carried on at a temperature below 250° F., and I prefer to use a temperature of about 225° F. This requirement also involves the question of viscosity of the material at the impregnating temperature, and I have found that a material suitable for this purpose must have a maximum viscosity at 225° F. of not over two poises, and preferably a minimum viscosity of .075 poises. That is, I have found no material suitable for this purpose having a viscosity of less than .075 poises at 225° F.

Fourth: For some purposes the material must be of such a nature as to prevent the growth of the fungi that produce decay.

A poise is the absolute unit of viscosity and may be defined as a force equivalent to one dyne per square centimeter. For comparative purposes it may be mentioned that water at ordinary temperatures has a viscosity of approximately .01 poises, while an 88% solution of glycerine in water at ordinary temperatures has a viscosity of approximately two poises.

It may be noted here that by the term "tracheids" I mean the microscopic cells which make up the greater part of the wood and which are known in wood structure as tracheids, fibre tracheids or libriform fibres. Also, by the term "pores" I mean the vessels and ducts of the wood.

I have found that montan wax not only fulfills all of these requirements and imparts to the wood the preservative and waterproof characteristics which are particularly desired, but that it also advan-

tageously changes the properties of the wood in certain other respects. A piece of wood which has been thoroughly impregnated with montan wax and the pores and tracheids thereof completely filled with the wax, is thereby rendered impervious to moisture, the growth of fungi in the wood is inhibited so that the wood will not decay, and furthermore, the wood so treated is an excellent electrical insulator, and it can be polished simply by cutting or abrading it to produce a smooth surface thereon.

The montan wax itself is highly waterproof so that when the pores and tracheids of the wood are filled with this wax it is impossible for water to work into the wood. This effectually eliminates any possibility of the wood shrinking or swelling. The presence of both air and moisture are required for the growth of the fungi that produce decay, and since the montan wax effectually seals the cells of the wood against the entrance of either air or moisture, it effectually preserves the wood.

While dry wood itself is a good insulator, it is impossible to keep it dry under normal conditions of use because of the hygroscopic nature of wood. The montan wax, however, excludes the water from the wood and it therefore preserves the wood in its most favorable condition for use as an insulator.

The ability of the impregnated wood to take a polish simply by making the surface thereof smooth, is an extremely important advantage in the manufacture of furniture and other wooden articles which are customarily varnished or finished in some similar manner. If the impregnation process is completed prior to the shaping of the article, the planing, turning, sanding, or other operations required to produce such shaping also produces a finish on the article, it simply being necessary to dust the surface of the work when it is completed, and to rub it somewhat if a higher polish is required. If desired, the manufacturing operations may be completed before the article is impregnated and the surface of the finished article may then be buffed to produce the finish or polish required.

Montan wax is a native mineral wax which is usually imported but is readily obtainable at a moderate expense and in large quantities. The usual source of supply is lignite or pyropissite from which the montan wax is extracted by means of solvents.

In impregnating the wood with this material the montan wax is melted and it may then be forced into the wood by either the open tank or pressure tank processes commonly used in impregnating wood with creosote oil. I prefer, however, to use the pressure process, and this process may be carried out with apparatus similar to that used in creosoting railroad ties. Very minor

modifications in such apparatus may be found desirable, such as steam jacketing the pipes, due to the fact that the montan wax is solid at normal temperatures. The treatment is facilitated by having the wood perfectly dry. The wood is placed in a pressure tank and is immersed in melted montan wax. The wax is then forced into the wood at a temperature preferably of from 225° to 250° F. and under a pressure preferably of from 125 to 200 pounds per square inch. The temperature, pressure, and length of time required to effect the desired impregnation will vary somewhat with the nature of the wood, the size of the pieces, and the degree of impregnation desired, as will readily be appreciated by those familiar with the processes of wood impregnation. In treating hard wood such as beech, birch and maple, I have obtained very satisfactory results by carrying on the impregnation at a temperature of 225° F. under a pressure of 200 pounds for three hours. The wood is then removed and allowed to cool. A considerable part of the montan wax is ejected from the wood during the process of cooling, but an ample quantity hardens in the pores and tracheids of the wood to produce the results above described.

If it is desired to recover a large part of the wax forced into the wood, this can be done by removing the pressure but maintaining the temperature high while the wood is allowed to drain. This will result in the pores and tracheids of the wood being partly emptied of the wax forced into them, while still leaving the cell walls thoroughly coated and the fibre of the wood effectually protected by the montan wax. When it is desired to retain a greater quantity of wax in the wood, the wood is allowed to cool down to a point near the solidification temperature, while still under pressure, before it is removed from the tank.

I find that I can produce a complete or through and through impregnation of the more common hard woods, such as beech, birch, maple and red oak. The woods which are naturally non-resistant take the treatment more readily than those which are more resistant to decay. The sap wood of spruce is very readily impregnated while the heart wood takes the treatment with more difficulty. This, however, is an advantage in treating spruce for use as poles, since the impregnation of the sap wood is sufficient to protect the pole from decay, with a minimum use of impregnating material. The montan wax, however, can be made to penetrate the heart wood of spruce to a very substantial extent.

The quantity of montan wax retained in the wood can be varied and the amount of material imprisoned or sealed within the wood will be controlled in accordance with the use to be made of the wood and considerations of economy. I prefer, however, to retain in the wood at least ten per cent of its own dry weight of montan wax. For most woods this means increasing its weight by at least two pounds per cubic foot of wood. The amount of montan wax held in the wood can be increased very substantially above these minimum figures, and for most purposes will be increased. In fact, I have found it possible to force into such woods as beech, birch and maple, over half of their own dry weight of montan wax. Even when a relatively small percentage of impregnating compound is to be retained in the wood it is preferable to force into it initially a much larger amount to secure uniform penetration, and then to allow the surplus material to drain off after the pressure has been removed, but while the temperature is maintained relatively high. This ensures a more uniform impregnation than could otherwise be obtained.

Preferably the wood to be treated should be thoroughly dry. It is important that any excess moisture be driven off before it is attempted to force wax into the wood. There is great danger, however, in boiling off this water that the wood will crack or "check." I have discovered that this difficulty can be effectually overcome by subjecting the wood to a light preliminary pressure of, say, from twenty to fifty pounds per square inch while the water is being evaporated. That is, the wood is immersed in the montan wax in the cylinder, as above described, heat being supplied to the wax to keep it at the desired temperature, and the pressure applied is regulated between the limits above mentioned, say, for example, at forty pounds per square inch, and is maintained at this point for the time required to drive off the water. This may be from one to four hours. It obviously would be more economical to drive off the water at atmospheric pressure, but this would involve danger of checking the wood. By applying a light preliminary pressure, as above described, the water is allowed to escape while the wood is protected from checking. When the water has been driven off the pressure is then raised to the desired degree necessary to force the montan wax into the wood. The length of time required for this purpose and the degree of pressure necessary may be determined by watching the action of the pressure gages and noting the point at which the wood "refuses" to take up further material.

After the wood has been impregnated there is no danger of its checking. In fact, when a checked piece of wood has been treated by this process it will not check further, but it will be preserved in the condition in which it is left by the treatment. This is

true even of thin cross sections of trees, such as those ordinarily used in museums for specimens and which practically always check.

- 5 The protection of the wood against checking is an exceedingly important practical advantage of this invention. The phenomenon of checking is only too well known to those familiar with the handling of wood, 10 and it is an important contributory cause to the decay of poles and timber exposed to the atmosphere, even when such poles or timber have been treated to preserve them. Telephone poles which have been butt treated and set up out-of-doors very often check or crack open above the ground, frequently splitting to the very heart of the pole. This admits water to the interior of the pole and allows decay to start at the butt of the pole 15 20 inside the area which has been treated with preservative.

The treatment with montan wax above described effectually prevents checking and preserves wood which has been checked, 25 partly by excluding moisture from the wood, and partly, also, due to the fact that when the montan wax has hardened in the wood it acts as a cement or binder. The wax itself does not expand or contract appreciably with atmospheric changes, and consequently, it holds the wood in a fixed and stable condition. None of the prior treatments of which I have been able to learn has this advantage.

- 35 While, as above stated, I have found montan wax best suited to the purposes of this invention, other substances having the characteristics above defined may be substituted for it. I have discovered that carnauba wax or candelilla wax possess some of the advantages of montan wax and that they may be used instead of montan wax in impregnating wood which is to be used for furniture and similar purposes. They both, however, are 40 45 open to the objection of being far more expensive than montan wax and are, at the present time, obtainable in only limited quantities. Furthermore, carnauba wax has the characteristic of shrinking greatly upon 50 cooling, and when a piece of wood impregnated with carnauba wax cools, the contraction of the wax compresses the wood so strongly that its shape is often changed.

It is also entirely possible to use other materials with montan wax to produce special effects. For example, in impregnating telephone poles, piles, posts, and other articles of wood which are to be used out-of-doors, such for example, as cross arms for telephone poles, piazza flooring, insulator pins, and the like, where the essential object is to make the wood waterproof and to preserve it, I find it not only feasible, but preferable, to combine a substantial percentage of creosote oil with the montan wax. This wax,

unlike most others, forms a very stable compound when mixed with creosote oil, and does not have the tendency to separate from the oil which most waxes, even including candelilla and carnauba do have, and which is extremely pronounced in the case of waxes of the paraffin series. A mixture of montan wax and creosote oil in the proportions of sixty percent by weight of the former to forty per cent of the latter form a composition which at normal temperatures has a waxy consistency, is highly waterproof, and is a good fungicide. This mixture is sufficiently fluid at 225° F. to flow readily into the tracheids of the wood during impregnation, the term "flow" being used to designate the movement of the liquid whether produced by pressure, capillarity, or otherwise. The surface of the impregnated wood will not soften or become tacky or greasy at temperatures below 140° F. Oil soluble coloring materials will also mix with this composition so that the wood can be colored as well as preserved. It has been definitely determined that .34 of a pound of grade *c* creosote oil per cubic foot of wood is sufficient to protect the wood from decay. I have found it entirely feasible to put in several pounds of creosote oil per cubic foot of wood in a mixture of the character just described. Furthermore, the toxicity of the solution may be even further increased by using other grades of creosote, such for instance, as that known commonly as "fraction 2" creosote oil which has three times the toxic strength of grade *c*. By impregnating a pole, post, or the like, with a mixture of this character the wood is not only given a toxicity which is ample to protect it from decay, but the toxic agent will be permanently held in the wood by the montan wax and prevented from exuding or oozing from the cells of the wood.

An especially important practical advantage of this feature of the present invention is that the relatively nonresistant woods, such for example, as spruce and the common southern yellow pines, can be treated by this process and thus made far superior to either chestnut or cedar for use as telephone poles, piling, posts, cross arms, insulator pins, and most of the uses for which the more resistant woods have been used almost exclusively heretofore. There is every reason to believe that a spruce pole treated by my process will outlast several times an untreated chestnut or cedar pole, and it can be produced at an expense which compares very favorably with the present price of cedar and chestnut poles in the eastern market.

In impregnating wood for furniture and similar articles, the montan wax may be mixed with oil soluble dyes to give the wood the desired color. Oils or waxes which will modify the polish or finish produced by the

montan wax may also be associated with it. The montan wax, or its equivalent, should predominate in any of these mixtures.

An especially important advantage produced by this invention in the finishing of furniture, flooring, and other wooden articles is that the structure of the wood is changed either throughout, or at least for a substantial depth, as distinguished from the 10 surface staining and finishing that is produced by the usual methods. Through the use of solvents, stains may be introduced into the wood for a very short distance, say for example, one-sixteenth of an inch, but no 15 impregnation of substantial depth is produced. By my process, however, the characteristics of the wood are changed for a substantial depth or even throughout the entire piece, depending upon the degree to 20 which the impregnation is carried. Consequently, a piece of furniture impregnated by this process will successfully withstand abuse that would ruin an article of furniture finished by the ordinary methods. 25 That is, bruises, nicks, and scratches in the finished surface of a piece of furniture impregnated with a composition in which montan wax predominates, can be easily shaved or buffed out, and the act of producing a smooth surface on the article also 30 reproduces the original finish. Similar injuries to a varnished surface would require the removal of the varnish from the entire surface and a complete refinishing of the article. Furthermore, my process is far more 35 economical both in labor and materials than the usual processes.

In treating wood for insulation, it may be desirable to mix transil oil or some other 40 insulating material with the wax, and I have found that compositions of this character can be used very satisfactorily, care, of course, being taken to see that any mixture used for impregnation comes within the requirements above specified.

It is further possible to mix with the montan wax a fire-proofing agent of the character used in rendering woods fire resistant. Sodium borate, for example, which has 50 been used heretofore for this purpose, may be associated with the wax. While these solid materials will not penetrate the tracheids of the wood and are largely strained out of the liquid montan wax as it is forced into the wood, they do lodge in the larger pores or vessels in the surface of the wood and thus protect it. Such a treatment is valuable for many purposes, as for example, in the treatment of shingles. The montan wax itself is 55 not readily inflammable, and in fact is ignited with some difficulty, so that the addition of a suitable fire-proofing agent makes a shingle treated by this process relatively 60 resistant to fire.

65 The protection of the wood against fire

can also be effected to advantage by introducing a solution of one of the water soluble, fire-retarding agents, such for example, as ammonium chloride, into the wood, and subsequently drying the wood and then impregnating it with montan wax. The wax effectually prevents the ammonium chloride from leaching out of the wood.

A very important practical advantage of this invention is that it makes many of the 70 cheap and relatively plentiful woods superior for many uses to woods that are not so abundant and are considerably more expensive. For example, it permits the use of spruce for telephone, telegraph, and electric light poles in place of chestnut and cedar. Beech, birch and maple can be treated by this process to resemble very closely mahogany and walnut, and they are given properties which actually make them superior 80 to mahogany and walnut in some respects. Locust is preferred at the present time for insulator pins, but a beech, birch or maple insulator pin treated in the manner above described is superior to locust for 85 this purpose, both in durability and in insulating properties. Many other advantages of this invention also will readily occur to those familiar with wood and wood products.

The present application is a continuation of my earlier applications Serial No. 626,818, filed March 22, 1923, and Serial No. 733,152, filed August 20, 1924, so far as the subject matter common to said applications and 100 the present case is concerned.

Having thus described my invention, what I desire to claim as new is:

1. An article of the character described consisting of wood impregnated for a substantial depth with a waxy material which remains hard and non-tacky at temperatures below 130° F. but is sufficiently fluid at 250° F. to be introduced into tracheids of the wood.

2. An article of the character described consisting of wood impregnated for a substantial depth with a waxy material which is hard and non-tacky at temperatures below 130° F., has a viscosity at 225° F. of between 110 .075 and 2.00 poises and is sufficiently fluid at 250° F. to flow into the tracheids of the wood.

3. An article of the character described consisting of wood impregnated for a substantial depth with a toxic preservative combined with a waxy material which remains hard and non-tacky at temperatures below 140° F. but is sufficiently fluid at 250° F. to be introduced into the tracheids of the wood.

4. An article of the character described consisting of wood impregnated with a toxic quantity of creosote oil combined with a proportion of a hard waxy material which prevents the oil from oozing from the surface 120

- of the wood at temperatures below 130° F., said waxy material becoming sufficiently fluid at 250° F. to flow into the tracheids of the wood.
5. An article of the character described consisting of wood carrying in the pores and tracheids thereof for a considerable depth a composition consisting chiefly of montan wax and a toxic preservative.
10. 6. An article of the character described consisting of wood impregnated with a toxic quantity of creosote oil and containing a sufficient proportion of montan wax associated with said oil to prevent the oil from oozing from the surface of the wood at temperatures below 130° F.
15. 7. An article of the character described consisting of wood impregnated with a mixture of creosote oil and montan wax in such proportions and quantity that the wood has a toxicity equivalent to at least three-tenths of a pound of grade C creosote oil per cubic foot of wood, and the quantity of montan wax being sufficient to prevent the creosote oil from oozing from the surface of the wood at temperatures below 130° F.
20. 8. An article of the character described consisting of wood impregnated for a substantial depth with a composition in which montan wax predominates.
25. 9. An article of the character described consisting of wood impregnated for a substantial depth with montan wax.
30. 10. That improvement in the process of treating wood to render it resistant to decay which consists in forcing into the pores and tracheids of the wood a melted mixture of a toxic preservative and a waxy substance which is hard and non-tacky at temperatures below 130° F. but becomes sufficiently fluid at 250° F. to flow into the tracheids of the wood, and allowing the wood to cool sufficiently to cause the mixture to harden within the pores and tracheids.
35. 11. That improvement in the process of treating wood which consists in forcing into the pores and tracheids of the wood a melted waxy material which is hard and non-tacky at temperatures below 130° F. but becomes sufficiently fluid at 250° F. to flow into the tracheids of the wood, and subsequently allowing the wood so treated to cool sufficiently to cause said waxy material to harden in the pores and tracheids thereof.
40. 12. That improvement in the process of treating wood which consists in impregnating the wood for a substantial depth with a composition in which montan wax predominates.
45. 13. That improvement in the process of treating wood which consists in impregnating the wood for a substantial depth with montan wax.
50. 14. That improvement in the process of treating wood containing excess water to impregnate it with a waxy substance which is hard at temperatures below 130° F. but becomes sufficiently fluid at 250° F. to flow into the tracheids of the wood, which consists in melting said substance, immersing the wood in the liquid so produced, driving the excess water out of the wood by heat transmitted to the wood through said liquid, maintaining a light preliminary pressure on said wood and liquid while said water is being driven off, and, after the desired amount of water has been driven out of the wood, increasing the pressure sufficiently to force said liquid into the pores and tracheids of the wood.
55. 15. The process of preventing checking in wood during the impregnation thereof with a waxy substance which is hard at temperatures below 130° F. but becomes sufficiently fluid at 250° F. to flow into the tracheids of the wood, which consists in melting said substance, immersing the wood in the hot liquid so produced, boiling the excess water out of the wood while so immersed by heat transmitted to the wood through said liquid, maintaining a pressure of from twenty to fifty pounds on the wood and liquid during said operation of driving off the water, and subsequently, after the excess water has been driven off, increasing the pressure on the wood and liquid sufficiently to force said liquid into the pores and tracheids of the wood.

JOSEPH R. COOLIDGE, III.